

## UNITED STATES PATENT OFFICE

2,504,593

## LIGHT-SENSITIVE ANTHRAQUINONE SULFONIC ACID PHOTOPRINTING MATERIAL CONTAINING A CUPRIC SALT

André Schoen, Stewartsville, N. J.; Alice Schoen, also known as Alice L. Schoen, executrix of said André Schoen, deceased, assignor to General Aniline & Film Corporation, New York, N. Y., a corporation of Delaware

No Drawing. Application May 18, 1946,  
Serial No. 670,852

8 Claims. (Cl. 95—7)

1

This invention relates to photoprinting material.

Many processes have been suggested for the production of photoprinting material, such processes differing principally in the chemical used as the light-sensitive element and in the manner of developing a dye image. The most widely known of these processes are those which are based upon the light sensitivity of aromatic diazo compounds, ferric salts and bichromates.

It is known that light-sensitive anthraquinone sulfonic acids and their salts, in the presence of oxidizable compounds, are reduced to the corresponding anthrahydroquinone when exposed to light. While it is possible to produce negative silver images by exposing paper coated with anthraquinone sulfonic acids and subsequently treating with silver salts, such a process is not practical because it requires four wet treatments of the exposed print.

It is an object of this invention to provide new photoprinting material employing light-sensitive anthraquinone sulfonic acids or their alkali-metal salts.

Another object is to provide a new process of photoprinting which does not require wet treatments for the development of the exposed print.

I have discovered that cupric salts are easily reduced to the cuprous state when exposed to light in the presence of a light-sensitive anthraquinone sulfonic acid or its alkali-metal salt, and that the cuprous salt formed can be converted by heating up to at least 100° C. to form a metallic copper image.

In one embodiment of my invention, a suitable base such as paper or film, and preferably gelatin-coated paper or film, is coated with an aqueous solution of the cupric salt, such as cupric formate, cupric lactate, cupric fluosilicate, cupric acetate, cupric aminoacetate, cupric gluconate, cupric sulfate, and the like, and a light-sensitive anthraquinone sulfonic acid or its salt, such as an anthraquinone 2,6-disulfonic acid, anthraquinone 2,7-disulfonic acid, anthraquinone 1,2-disulfonic acid, anthraquinone-2-sulfonic acid, and the like, or alkali-metal salts thereof. Of the cupric salts mentioned above, cupric formate is preferred since it is more easily reduced to cuprous formate which is readily converted to metallic copper. After drying, the coated carrier is exposed to light in contact with an original to be reproduced. The anthraquinone sulfonic acid is reduced to the corresponding anthrahydroquinone, which in turn reduces the cupric salt to the cuprous state. The exposed carrier is then heated

2

to an elevated temperature, for example, from 100 to 170° C., whereupon a metallic copper image is formed.

In another embodiment the carrier coated with the light-sensitive anthraquinone sulfonic acid and the cupric salt is employed in reflex printing. Prints made according to this invention have a red to brown color, possess good white backgrounds, good contrast, and excellent opacity to ultra-violet, violet, and blue light, permitting a wide range of printing speeds when used as transition prints without danger of overexposure. The process has great simplicity due to the advantages of dry development and fixing.

15 The addition of a mild reducing agent such as glycerine, sorbitol, etc., to the coating solution gives increased sensitivity and higher densities.

The keeping quality of the coated paper or film, and the permanency of the developed print 20 can be improved if the paper or film, after being sensitized, is given a coating of a water-resistant compound, such as paraffin.

The following examples illustrate methods of carrying out the present invention, but it is to be 25 understood that these examples are given by way of illustration and not of limitation.

## Example 1

30 Gelatin coated film is treated with a coating solution of:

10 g. cupric formate  
2 g. anthraquinone 2,6-disodium sulfonate  
100 cc. water,

35 and dried. The coated film is then exposed to light under an original to be reproduced, the exposed film is heated to 130–140° C. for three minutes, and a dark brownish-red negative print of excellent contrast is obtained.

40 When 6 cc. of glycerine is added to the above coating solution, and the coated film is exposed to light and heated as above, the image is darker.

## Example 2

45 A gelatin coated paper is treated with the following coating solution

15 g. cupric formate  
2 g. anthraquinone 2,7-disodium sulfonate  
20 cc. glycerine  
100 cc. water,

and dried. The paper is exposed to light under a negative, and then heated for five minutes at 130° C. whereupon a brownish-black positive of 50 excellent contrast is formed.

*Example 3*

A gelatin coated film is treated with the following coating solution

13 g. cupric formate  
2 g. anthraquinone 2,6-disodium sulfonate  
10 cc. glycerine  
100 cc. water,

and dried. The film is exposed to light over a positive, and then heated at 170° C. for five seconds, whereupon a dark brownish-red negative of excellent contrast is obtained.

*Example 4*

A gelatin coated paper is treated with the following coating solution

6 g. cupric lactate  
2 g. anthraquinone 2,6-disodium sulfonate  
10 cc. glycerine  
100 cc. water,

and dried. The coated paper is exposed to light under a negative, and then heated at 100° C. for two hours. A brown colored print is obtained.

*Example 5*

Paper is treated with the following coating solution

15 g. cupric fluosilicate  
2 g. anthraquinone 2,6-disodium sulfonate  
10 cc. glycerine  
100 cc. water,

and dried. The coated paper is exposed to light under a negative, and then heated at 150° C. for one minute. A red-brown image is obtained.

*Example 6*

A gelatin coated film is treated with the following coating solution

15 g. cupric aminoacetate  
2 g. anthraquinone 2,6-disodium sulfonate  
10 cc. glycerine  
100 cc. water,

and dried. The coated film is exposed to light under a negative, and heated to 120° C. for fifteen minutes. A reddish-brown colored image is obtained.

*I claim:*

1. A photoprinting material comprising a light-sensitive layer on a suitable carrier containing cupric formate and a member of the group consisting of anthraquinone 2,6-disulfonic acid, anthraquinone 2,7-disulfonic acid and the alkali-metal salts thereof.

2. A photoprinting material comprising a light-sensitive layer on a suitable carrier contain-

ing cupric formate, a mild reducing agent and a member of the group consisting of anthraquinone 2,6-disulfonic acid, anthraquinone 2,7-disulfonic acid and the alkali-metal salts thereof.

5. 3. A photoprinting material comprising a light-sensitive layer on a suitable carrier containing cupric formate and a member of the group consisting of anthraquinone-2,6-disulfonic acid and its alkali-metal salt.

10 4. A photoprinting material comprising a light-sensitive layer on a suitable carrier containing cupric formate, glycerin and a member of the group consisting of anthraquinone-2,6-disulfonic acid and its alkali-metal salt.

15 5. A dry process of reproducing an original which comprises exposing to light a light-sensitive layer on a suitable carrier containing a cupric formate and a member of the group consisting of the anthraquinone-2,6-disulfonic acid, anthraquinone-2,7-disulfonic acid and the alkali metal salts thereof in contact with an original to be reproduced, and heating the thus exposed light-sensitive layer to from 100° C. for 2 hours to 170° C. for 5 seconds.

20 6. A dry process of reproducing an original which comprises exposing to light a light-sensitive layer on a suitable carrier containing a cupric formate, a mild reducing agent and a member of the group consisting of the anthraquinone 2,6-disulfonic acid, anthraquinone-2,7-disulfonic acid and the alkali-metal salts thereof in contact with the original to be reproduced and heating the thus exposed light-sensitive layer to from 100° C. for 2 hours to 170° C. for 5 seconds.

25 7. The process in accordance with claim 5 in which the light-sensitive anthraquinone sulfonic acid is anthraquinone-2,6-disulfonic acid.

8. The process in accordance with claim 6 in which the light-sensitive anthraquinone sulfonic acid is anthraquinone-2,6-disulfonic acid, and the reducing agent is glycerin.

ANDRÉ SCHOEN.

## REFERENCES CITED

45 The following references are of record in the file of this patent:

## UNITED STATES PATENTS

50 Number Name Date  
1,843,822 Kogel Feb. 2, 1932

## FOREIGN PATENTS

Number Country Date  
55 506,413 Germany Sept. 4, 1930  
702,183 France Jan. 19, 1931